

stated, is to provide an alloy for use in electrical instruments, such as temperature controls and in instruments which are idle for long periods but must have reliable contacts when called upon to function, and which contact temperature, be it proof against deleterious atmospheric influences, other influences which would otherwise render them unreliable and uncertain or inoperative. As a result of a temperature controlled instrument of the character referred to, reference may be made to thermastic switches for fire or other alarm circuits which connect and disconnect exposed to the oxidizing effects of air or steam, and in many cases to the corrosive influences of nitric and sulphuric acid vapors or chlorine or other gases.

Heretofore, so far as I am aware, no contacts for instruments of such type have been made which have been successful in meeting in full the regulations of the Insurance Underwriters' Laboratories requiring such contacts to be proof against oxidation and corrosion. Consequently, it has been necessary in practice to employ instruments which are satisfactory only to a certain degree, but fall short of what a theoretically and practically reliable instrument should be.

As a result of long and extensive experiments I have succeeded in producing and perfecting an alloy which is eminently suitable for the manufacture of contacts for such class of instruments, and which alloy meets all the requirements of the Insurance Underwriters' Laboratories regulations, that is to say, it is of low melting and high electrical conductivity and proof against the deleterious action of air or steam and against the corrosive action of the vapors of nitric, sulphuric and other acids, and of chlorine and other gases, and which, therefore, while of no particular value for use in the make and break instruments

stated, but which must be proof against such influences and which is reliable in action, although idle for long periods.

The particular object of my invention, therefore, is to provide an alloy which will fully meet the Insurance Underwriters' Laboratories regulations and which, in addition to its value for use in instruments of the character mentioned, is preferred to, is adapted for highly efficient use in telephone, telegraph and radio instruments, and in which high conductivity and low resistance are important factors, such as in telephone, telegraph and radio instruments and circuits.

In carrying my invention into practice, I provide a new alloy for the purposes described, comprising gold, approximately 20%, and silver, approximately 70%. These proportions may be varied to some slight degrees dependent upon the sources and characteristics of the metals themselves, but the proportions given are desirable and essential under general conditions. Since proportions, for example, provide an alloy of suitable medium hardness, whereas the metal alone in the same proportions materially different from those given will be of insufficient hardness or be objectionable as not meeting required conditions in other respects. The alloy of gold and silver in the stated proportions is inexpensive to produce, can be readily welded or welded or machined for making welded or staked contacts in instruments, is proof against oxidation and corrosion, under the influences of air, steam, water, nitric or sulphuric acids or chlorine or other gases, a quality given by the gold and silver proportions employed, and has low electrical resistance and high electrical conductivity, a quality given it by the silver in the proportion employed. The qualities mentioned make it particularly valuable for use as electrical contacts in telephone, telegraph and radio instruments where small currents are employed, and high conductivity, low resist-

85  
20 switches controlling fire alarm or similar apparatus. Such devices, when used in factories and various industrial plants, are exposed to the oxidizing or corrosive influences of air, steam, water, nitric, sulphuric or other acid vapors, and chlorine or other gases, and are liable to be functionally impaired, if not sufficiently resistant against them. Contacts made of my novel alloy are proof against such influences or conditions, and against them that they may be exposed to them for very long periods without being functionally or physically impaired to such a degree as to prevent them from making certain and reliable contact. 90  
25 The contact terminals may be made and applied for use in any suitable way, I do not limit myself in this particular, but, for purposes of exemplification, I may state that in the use of the alloy for the contact terminals of a thermostatic circuit closing device employing a metallic contact strip having a contact terminal at its free end engageable with a pointed contact terminal on the end of a contact pin or screw, the terminal or the strip may be in the form of a disk or button welded or fastened to the strip, while the contact terminal on the pin or screw may be welded or otherwise fastened to the strip. These terminals may be quite small and therefore, inexpensive, and by constructing them to have a wiping contact on a circuit closing and opening, will not only be free of adhering oxidation or corrosion, but also will cut through a dust, dirt or grease coating and thereby make positive contact. 100  
30 In addition, this composition of gold and silver in the stated proportions, produces an alloy which is of particular value as a circuit closing device, in that the pointed contact terminal has a wiping engagement with a metallic contact strip, as the alloy is of just the right degree of hardness and strength to allow such wiping contact to be made under considerable pressure without injury to the contacts, while allowing any adhering film 105  
35 110  
40 115  
45 120  
50 125  
55 130  
60 135  
65 140